

## UNITED STATES PATENT OFFICE

2,208,517

## PRODUCTION OF DIARYL COMPOUNDS

Carl F. Prutton, Cleveland, Ohio, assignor to The Dow Chemical Company, Midland, Mich., a corporation of Michigan

No Drawing. Application July 20, 1935,  
Serial No. 32,447

3 Claims. (Cl. 260—670)

This invention relates to improvements in processes for producing diphenyl and higher diaryl compounds by the pyrolysis of benzene and its homologues, or mixtures thereof. 5  
One of the difficulties commonly associated with processes in which benzene hydrocarbons are heated at high temperatures is the formation of the carbon on the heating surfaces. Such carbon formation causes a loss of materials in 10 process, while the carbon deposits so formed interfere with the transfer of heat and frequently cause interruptions of the process for removing carbon accumulations which obstruct the apparatus.

15 In apparatus for pyrolyzing benzene hydrocarbons, it is desirable to employ iron or steel as the material of construction wherever it can be used without detriment. It is known, however, that in the pyrolysis of hydrocarbons at high 20 temperatures, e. g., in the range of approximately 500° to 900° C., iron promotes the formation of carbon. Particularly, in connection with the pyrolysis of benzene hydrocarbons for the formation of diphenyl and related diaryl compounds 25 it has been found that much trouble is encountered due to the formation of carbon when the process is carried out in iron apparatus, as reported in the literature (cf. Smith and Lewcock, J. Chem. Soc. 101, 1453—1459; Zanetti and 30 Egloff, J. Ind. Eng. Chem. 9, 350—356). The formation of carbon deposits seriously interferes with the regular and continuous operation of the method, so much so that it has generally been regarded as impracticable to use apparatus of 35 wrought iron or carbon steel, particularly tubular apparatus, in a commercial process for pyrolyzing benzene in the usual temperature range of about 650°—850° C., because the apparatus would rapidly become filled with carbon and frequent shutdowns would be necessary for cleaning 40 out the carbon. Various proposals have been made for avoiding or overcoming the aforesaid difficulty, among which it has been suggested to provide special coatings or linings on ordinary 45 steel apparatus which inhibit or reduce the formation of carbon, or to introduce along with the vapors of the benzene hydrocarbon a foreign substance which has the effect of preventing or counteracting the formation of carbon.

50 I have now found a much simpler method than those heretofore proposed, by which carbon formation in the pyrolysis of benzene and benzene hydrocarbons, when carried out in apparatus of iron or carbon steel, can be greatly reduced, so 55 that it does not interfere materially with the con-

tinuous operation of the process. The invention is based upon my discovery that a preliminary carburizing treatment of the iron surfaces of the pyrolyzing apparatus serves to suppress the catalytic action of iron in causing formation of 5 carbon in the apparatus subsequently when benzene hydrocarbons are exposed to a pyrolyzing temperature therein.

It is among the objects of the invention to provide a method of pyrolyzing benzene hydrocarbons, wherein the formation of carbon is 10 greatly reduced, or even substantially prevented, so that a process employing the method can be carried on continuously for long periods of time without interruptions caused by carbon accumulations. Another object is to enable the use of 15 wrought iron or ordinary carbon steel as structural material in apparatus for carrying out the aforementioned pyrolytic reaction. Other objects and advantages will appear in the following 20 description in which the invention is fully set forth and particularly pointed out in the claims.

In connection with experiments with the pyrolysis of benzene vapors in the temperature range of 650° to 850° C., in which the vapors were 25 passed through heated tubes of wrought iron or carbon steel, it was found that within a few hours at most the tubes would become practically blocked with carbon. This result occurred irrespective of the purity of the benzene, or of the 30 rate of vapor flow, the carbon formation, of course, being the more rapid the higher the temperature within the range stated. The accumulation of carbon in the apparatus necessitated 35 frequent shutdowns for cleaning out the carbon and indicated the practical impossibility of using ordinary iron or steel tubes in commercial apparatus for making diphenyl and diaryl compounds by pyrolyzing benzene hydrocarbons, inasmuch as a commercial process would be required to operate continuously over considerable 40 periods of time.

I observed, however, that carbon was formed less rapidly in tubes which had been previously 45 used for pyrolyzing benzene until filled with carbon and from which the carbon had been cleaned out. In particular, I found that if care was taken not to scrape the surfaces of the iron tube in removing the carbon, simply blowing out the loose carbon and lightly brushing the surfaces 50 to remove adhering particles, even better results were obtained in the reduction of carbon formation when the cleaned tubes were later used again in the pyrolysis. Apparently a layer of iron carbide had been formed on the exposed 55

iron surfaces, which, once produced, prevented or counteracted further catalytic action of the iron itself in causing the carbon formation. In order to demonstrate the effectiveness of a preliminary carburizing of the iron tubes prior to using the same for pyrolyzing benzene, the following experiments were conducted:

*Example 1*

- 10 A 1-inch mild steel tube was carburized by heating to about 900° C. for 9 hours while packed with charcoal. The carburized tube was then placed in a furnace, and connected at one end with a source of supply for benzene vapors, and at the other end with a condenser. The tube was heated and benzene vapors passed therethrough at a rate corresponding to the vaporization of 5 cubic centimeters per minute, the temperature inside the tube reaching a maximum of approximately 750° C. The hot vapors were condensed, and the unreacted benzene in the condensate was again vaporized and recirculated through the apparatus. After 9 hours of continuous operation the test was discontinued, although no obstruction to the passage of benzene vapors had occurred. A small amount of loose carbon was found in the tube, amounting to 4.5 grams. The percentage yield of diphenyl in this run was 62 per cent. In a check run under the same conditions, except that an uncarburized tube otherwise similar to the first one was used, the tube was completely stopped with carbon at the end of 5 hours, and 41.2 grams of carbon were removed from the tube after the run was stopped, while the yield of diphenyl was only 33 per cent.

*Example 2*

- 40 In a similar experiment a 1-inch steel tube was used, which had been case-hardened on the inner surface by heating with sodium cyanide at about 900° C. for about 9 hours. Benzene vapors were circulated through the tube at the same rate as before for 9 hours, while heating the same to a maximum temperature of about 750° C. No stoppage of vapor flow occurred during the time. At the end of the run a quantity of 45 7.2 grams of carbon was removed from the tube.

I have found that similar tubes which had been thoroughly carburized on the inner surface can be used continuously for as long as 450 hours or more for pyrolyzing benzene at a temperature between 700° and 750° C. without formation of

sufficient carbon therein to cause obstruction to the passage of vapors therethrough, whereas without such preliminary carburizing treatment they would have been completely stopped with carbon in a few hours.

5 My invention thus makes possible the commercial production of diphenyl and related diaryl compounds, and mixtures thereof, by pyrolysis of benzene hydrocarbons carried out in tubular or equivalent apparatus made of iron or carbon steel. The pyrolyzing tube or reactor parts need only be thoroughly carburized on the surfaces which are to be exposed to the hydrocarbon vapors at a pyrolyzing temperature. Such carburization may be done in any of the ways known to the art, to produce on the iron a surface layer consisting chiefly or substantially of iron carbide.

10 Other modes of applying the principle of my invention may be employed instead of those explained, change being made as regards the method herein disclosed, provided the step or steps stated by any of the following claims or the equivalent thereof be employed.

15 I therefore particularly point out and distinctly claim as my invention:

20 1. In a method of pyrolyzing benzene hydrocarbons, the improvement which consists in preventing or reducing the formation of carbon by heating the benzene hydrocarbon vapors at a diaryl-forming temperature in an apparatus of 25 iron or carbon steel, the surfaces of which exposed to contact with the vapors have been previously subjected to a carburizing treatment for a time sufficient to form a carbide coating thereon.

25 2. In a method of making diphenyl, the improvement which consists in preventing or reducing the formation of carbon by heating benzene vapors at a diphenyl-forming temperature in an apparatus of iron or carbon steel, the surfaces of which exposed to contact with the vapors have been previously subjected to a carburizing treatment for a time sufficient to form a carbide coating thereon.

30 3. In a method of pyrolyzing benzene hydrocarbons to produce diaryl compounds, the step which consists in passing the hydrocarbon vapors at a temperature between 650° and 850° C. over heated surfaces of iron or carbon steel which have been subjected to a carburizing treatment for a time sufficient to form a carbide coating thereon.

35 45 50 CARL F. PRUTTON.